# EUROPEAN PATENT SPECIFICATION

(11) **EP 3 112 051 B1**
(45) Date of publication and mention of the grant of the patent: **15.05.2019**
(21) Application number: 15754485.9
(22) Date of filing: 30.01.2015
(51) Int. Cl.: B22D 11/115

(54) **CONTINUOUS STEEL CASTING METHOD**
VERFAHREN ZUM KONTINUIERLICHEN STAHLGIESSEN
PROCÉDÉ DE COULAGE D'ACIER EN CONTINU

(30) Priority: 25.02.2014 JP 2014034130
(43) Date of publication of application: 04.01.2017
(73) Proprietor: Nippon Steel & Sumitomo Metal Corporation, Tokyo 100-8071 (JP)
(72) Inventor: OKADA, Nobuhiro, Tokyo 100-8071 (JP)
(74) Representative: J A Kemp
(86) International application number: PCT/JP2015/052627
(87) International publication number: WO 2015/129382

(56) References cited:
- EP-A1- 1 623 777
- JP-A- 2003 236 644
- JP-A- 2004 322 120
- JP-A- 2006 082 092
- JP-A- 2012 166 209
- JP-B2- 5 310 205
- KUNSTREICH S: "ELECTROMAGNETIC STIRRING FOR CONTINUOUS CASTING (PART 2)//BRASSAGE ELECTROMAGNETIQUE POUR COULEE CONTINUE (PARTIE 2)", REVUE DE METALLURGIE - CAHIERS D'INFORMATIONS TECHNIQUES, REVUE DE METALLURGIE. PARIS, FR, vol. 100, no. 11, 1 November 2003 (2003-11-01), pages 1043-1061, XP001046813, ISSN: 0035-1563, DOI: 10.1051/METAL:2003113
- CHRISTER CARLSSON ET AL: "Melhoramento na qualidade e produtividade no lingotamento de placa lll por vibração e parada eletromagnética / Improved quality and productivity in slab casting by electromagnetic braking and stirring", TECNOLOGIA EM METALURGIA, MATERIAIS E MINERAÇ 41ST STEELMAKING SEMINAR - INTERNATIONAL; MAY 23RD TO 26TH, 2010, AMAN - ACADEMIA MILITAR DAS AGULHAS NEGRAS - RESENDE, RJ, BRAZIL, ASSOCIAÇÃO BRASILEIRA DE METALURGIA, MATERIAIS E MINERAÇÃO, SÃO PAUL, vol. 8, no. Suppl, 1 January 2011 (2011-01-01), pages 1-15, XP008176633, ISSN: 2176-1515
- KEISUKE FUJISAKI: "In-Mold Electromagnetic Stirring in Continuous Casting", IEEE TRANSACTIONS OF INDUSTRY APPLICATIONS, vol. 37, no. 4, 2001, XP002773448,
- LEONARDO B. TRINDADE ET AL.: 'Numerical Model of Electromagnetic Stirring for Continuous Casting Billets' IEEE TRANSACTIONS ON MAGNETICS vol. 6, no. 38, November 2002, ISSN 0018-9464 pages 3658 - 3660, XP001141046

## Description

### Technical Field

This invention relates to a method for optimally operating an electromagnetic stirrer disposed in a mold, to continuously cast steel.

### Background Art

One of the main causes of making the quality of a superficial slab manufactured by continuous casting deteriorate is a pinhole defect. Such a pinhole defect is generated by such Ar gas as to be brown into a submerged nozzle for suppressing blocking up of the submerged nozzle in continuous casting, to enter molten steel in a mold, and to be captured by a solidified shell.

It is effective to dispose an electromagnetic stirrer in a mold as a method for suppressing pinhole defects. Operation factors of this electromagnetic stirrer include the flow velocity of molten steel, a submerged nozzle, a molten steel throughput and the Lorentz force.

For example, the following arts are disclosed as they make these operation factors within proper ranges.

For example, Patent Literature 1 discloses the art of making the flow velocity of electromagnetic stirring at a meniscus 10 to 60 cm/s in order to decrease the generation rate of defects on a surface of a slab to be obtained.

Patent Literature 2 discloses the art of making surface defects on a slab due to attachment of air bubbles to a solidified shell, a certain count or less, using parameters such as a distance between an immersion nozzle and a long side of a mold, a length in a casting direction of a molten steel discharge opening of the immersion nozzle, a throughput quantity of molten steel, and the magnetic field density at a solidification interface. Patent Literature 2 describes that the distance between the immersion nozzle and a long side of the mold is controlled by changing the shape of the immersion nozzle and the shape of the mold.

Patent Literature 3 discloses the art of imparting electromagnetic forces so that the average value of an electromagnetic force in a direction parallel to a major side of a casting mold is 3,000 to 12,000 N/m³, the localized value of an electromagnetic force in a direction parallel to a minor side of the casting mold is -2,000 to 2,000 N/m³, and the localized value of an electromagnetic force in a perpendicular downward direction is -1,000 to 1,000 N/m³ in order to accelerate float of bubbles of Ar gas and avoid contamination of mold powder into molten steel.

Application of the above described arts disclosed in Patent Literatures 1 to 3 suppresses pinhole defects to some extent. However, pinhole defects do not completely disappear. Users more and more strictly demand the quality of surfaces of steel plates, which necessitates an art of further suppressing pinhole defects.

An electromagnetic stirrer is a device that is the most effective for suppressing pinhole defects in continuously steel casting. In the above described arts disclosed in Patent Literatures 1 to 3, electromagnetic forces generated by electromagnetic stirrers and proper ranges of the flow velocities of molten steel generated by the electromagnetic forces are also examined in detail.

Here, an electromagnetic stirrer is a device that generates the Lorentz force in molten steel in a mold, to make the molten steel flow. This Lorentz force is generated only in molten steel having conductivity, but not generated in what generally called insulators, which have extremely low conductivity such as air bubbles of Ar gas.

Thus, air bubbles of Ar gas move relatively in the opposite direction to the movement of molten steel in a mold. That is, an electromagnetic force generated by an electromagnetic stirrer also includes a negative component that gathers air bubbles of Ar gas on a superficial slab as shown in FIG. 8, to increase pinhole defects.

This component of an electromagnetic force, gathering air bubbles of Ar gas which are included in molten metal on a superficial slab is called "electromagnetic repulsion" or "electromagnetic Archimedes force", which is described in Non Patent Literature 1 in detail. In FIG. 8, 1 represents a wall surface of a mold, 2 represents a solidified shell, 3 represents a solidification interface and 4 represents an air bubble of Ar gas; the arrow pointing the top from the bottom on the page represents the Lorentz force, and the arrow pointing the bottom from the top on the page represents electromagnetic repulsion. Non Patent Literature 2 discloses thermal fluid simulation in view of Lorentz force density acting on molten steel in continuous casting.

JP 5 310205 discloses a method for controlling flow of molten steel in a casting mold, in which a cast slab with a superior surface property is stably manufactured while avoiding contamination of mold powder into the molten steel by quantitatively controlling the manner of an electromagnetic force being formed in an electromagnetic stirring device, and thereby more effectively accelerating float of argon bubbles.

JP 2006 082092 discloses a method to properly carry out the control of the flow of molten steel by properly selecting the frequency of the moving magnetic field according to casting conditions when carrying out the continuous casting while controlling the flow of molten steel in a casting mold by applying the electromagnetic force caused by the moving magnetic field to the flow discharged from an immersed nozzle.

### Citation List

### Patent Literature

Patent Literature 1: JP H6-605A
Patent Literature 2: JP 2007-216288A
Patent Literature 3: JP 2010-240687A

### Non Patent Literature

Non Patent Literature 1: Tetsu-to-hagané, Vol. 83 (1997), No. 1, pp. 30-35
Non Patent Literature 2: K. Takatani: ISIJ International, Vol. 43, 2003, No. 6, pp. 915-922

### Summary of Invention

### Technical Problem

A problem to be solved by this invention is that in conventional arts, there is no concept of determining preferable conditions for electromagnetic stirring, focusing on electromagnetic repulsion generated by an electromagnetic stirrer, in electromagnetic stirring of molten steel in a mold upon continuously casting steel.

### Solution to Problem

An object of the present invention is to determine the best current frequency of an electromagnetic stirrer so as to make electromagnetic repulsion generated upon electromagnetic stirring of molten steel in a mold as low as possible, to further suppress pinhole defects.

The present invention was made based on the results of the inventor's study described below, and its primary feature is: in continuously casting steel using a mold and an electromagnetic stirrer, the mold being equipped with the electromagnetic stirrer, obtaining a relationship between effective Lorentz force density F (N/m³) that is calculated by the following formula, and current frequency (Hz) of the electromagnetic stirrer, and using current frequency of the electromagnetic stirrer such that the effective Lorentz force density F is within a range of Fmax to 0.9 Fmax wherein Fmax is a maxmum value of the effective Lorentz force density F, wherein F = Lx - α·Ly, and in this formula, Lx (N/m³) is an average value of Lorentz force density components in a direction parallel to a long side of the mold within existence of an iron core, the iron core being a component of the electromagnetic stirrer, Ly (N/m³) is an average value of Lorentz force density components in a direction parallel to a short side of the mold within existence of the iron core, and α is a coefficient indicating bad influence of electromagnetic repulsion and is within the range of 3 to 7.

In the above described present invention, the best current frequency of the electromagnetic stirrer is determined so as to make electromagnetic repulsion generated upon electromagnetic stirring of the molten steel in the mold as low as possible. Thus, it can be suppressed as far as possible to gather air bubbles of Ar gas on a superficial slab.

### Advantageous Effects of Invention

According to the present invention, pinhole defects can be further suppressed compared with methods for continuously casting steel using conventional arts because it can be suppressed as far as possible to gather air bubbles of Ar gas on the superficial slab.

### Brief Description of Drawings

FIG. 1 is a view to explain a mold and an electromagnetic stirrer used in the method for continuously casting steel of the present invention, seen from the top of the mold.
FIG. 2 shows the distribution of Lorentz force density at the center position of an iron core in a slab drawing direction, obtained by numerical simulation.
FIG. 3 shows the relationship between average values Lx of Lorentz force density components in the direction parallel to a long side of the mold within the existence of the iron core of the electromagnetic stirrer, and current frequencies.
FIG. 4 shows the relationship between average values Ly of Lorentz force density components in the direction parallel to a short side of the mold within the existence of the iron core of the electromagnetic stirrer, and current frequencies.
FIG. 5 shows the relationship between Ly/Lx and current frequencies.
FIG. 6 shows the findings of change in the number of pinholes per unit area (number/m²) on a solidification interface according to current frequencies, based on numerical analysis.
FIG. 7 shows frequency dependency of effective Lorentz force density F in a case where a coefficient α that indicates bad influence of electromagnetic repulsion is 5.
FIG. 8 is a view to explain electromagnetic repulsion.

### Description of Embodiments

The present invention realizes the object of determining the best current frequency of an electromagnetic stirrer so as to make electromagnetic repulsion generated upon electromagnetic stirring of molten steel in a mold as low as possible, to further suppress pinhole defects.

Upon operating a continuous casting machine where a mold is equipped with an electromagnetic stirrer, the inventor found as a result of his specific study on electromagnetic repulsion generated in the mold that pinhole defects can be reduced by suppressing the electromagnetic repulsion.

Then, as a result of the inventor's further study on a method for applying an electromagnetic force which suppresses the electromagnetic repulsion so as to keep bubbles of Ar gas away from the vicinity of a solidification interface, it turned out that there exists a proper current frequency upon applying the electromagnetic force.

The mold and the electromagnetic stirrer used in the above studies are same as those described in Patent Literature 3, which have ordinary shapes and polarities as shown in FIG. 1 when the mold is seen from the top. In FIG. 1, 11 represents a copper mold (hereinafter may be referred to as a mold), 12 represents a submerged nozzle, 13 represents an electromagnetic stirrer, 13a represents an iron core constituting the electromagnetic stirrer 13, 13aa represents a teeth part formed on the iron core 13, and 13b represents a winding that is wound around the outer circumference of the iron core 13a.

FIG. 2 shows the distribution of Lorentz force density at the center position of the iron core in a slab drawing direction, obtained by numerical simulation. Here, Lorentz force density represents an electromagnetic force per unit volume of molten steel (N/m³).

The distribution of Lorentz force density shown in FIG. 2 resulted from the numerical simulation under the conditions where the size of a slab was 1200 mm in width × 250 mm in thickness, a copper plate forming the mold was 25 mm in thickness, and the conductivity of the mold was 1.9 × 10⁷ S/m.

The distribution of Lorentz force density shown in FIG. 2 is the distribution of stirring the molten steel in the mold counterclockwise. The large Lorentz force along the direction of a long side of the mold 11 is generated in the vicinity of the wall surface of the mold 11.

As is clear from FIG. 2, the above described Lorentz force along the wall surface of the mold also includes a lot of components directed toward the inside of the mold. Such a kind of the Lorentz force directed toward the inside of the mold functions as electromagnetic repulsion directed toward the wall surface of the mold for bubbles of Ar gas. That is, the electromagnetic repulsion transmits bubbles of Ar gas to the vicinity of the interface of a solidified shell, and pinhole defects are increased.

Distribution of the Lorentz force density does not change even if an EMS (Electro-Magnetic Stirrer) current value becomes larger. That is, in a case where the current value of an electromagnetic stirrer is made to be larger, to speed up the flow velocity, the effect of suppressing pinhole defects can be obtained by a cleaning effect on pinholes captured by the interface of a solidified shell; on the other hand, electromagnetic repulsion makes bubbles of Ar gas moving to the interface of the solidified shell increase and thus, pinhole defects increase.

As a result of the inventor's study, it was very effective for reducing the components of the Lorentz force directed toward the inside of the mold to change the current frequency of the electromagnetic stirrer, as described below.

FIG. 3 shows the relationship between average values Lx (N/m³) of the Lorentz force density components in the direction parallel to a long side of the mold within the existence of the iron core of the electromagnetic stirrer, and current frequencies (Hz). The above described values Lx in the direction parallel to a long side of the mold were calculated assuming that the Lorentz force in the direction same as the revolution of the molten steel due to electromagnetic stirring was positive and the Lorentz force in the direction opposite thereto was negative.

Specifically, the values Lx were calculated assuming that the Lorentz force density in the left direction on the page of FIG. 2 was positive and the Lorentz force density in the right direction thereon was negative in the area of the page upper than the center of a short side of the mold; and the Lorentz force density in the right direction on the page was positive and the Lorentz force density in the left direction on the page was negative in the area of the page lower than the center of a short side of the mold.

According to FIG. 3, the maximum of the above described value Lx in the direction parallel to a long side of the mold exists in the range of 2.3 to 2.5 Hz in current frequency; and the current frequency should be selected out of this range of 2.3 to 2.5 Hz for making the stirring flow velocity maximum.

FIG. 4 shows the relationship between average values Ly (N/m³) of Lorentz force density components in the direction parallel to a short side of the mold within the existence of the above described iron core, and current frequencies (Hz). The above described values Ly in the direction parallel to a short side of the mold were calculated assuming that the Lorentz force density directed toward the inside of the mold was positive and the Lorentz force density directed toward the outside of the mold was negative.

Specifically, the values Ly were calculated assuming that downward Lorentz force density that was leaving away from the wall surface in a long side of the mold was positive in the area of the page of FIG. 2 upper than the center of a short side of the mold, in and upward Lorentz force density that was leaving away from the wall surface in a long side of the mold was positive in the area of the page lower than the center of a short side of the mold.

That is, the above described value Ly in the direction parallel to a short side of the mold represents a component of the Lorentz force density which makes the molten steel in the mold move from the wall surface in a long side of the mold to the center of a short side, and represents electromagnetic repulsion which makes bubbles of Ar gas move to the wall surface of the mold. As is clear from FIG. 4, as the current frequency of the electromagnetic stirrer is high, the above described value Ly in the direction parallel to a short side of the mold gets large.

FIG. 5 shows the ratio Ly/Lx of the above described value Ly in the direction parallel to a short side of the mold to the above described value Lx in the direction parallel to a long side of the mold. As is seen from FIG. 5, as the value of Ly/Lx is small, the electromagnetic repulsion component in the Lorentz force density generated in the molten steel in the mold is a little.

As is seen from FIGS. 4 and 5, it is effective for reducing electromagnetic repulsion to decrease the current frequency. As is seen from FIG. 3, it is necessary for securing the stirring flow velocity originating from electromagnetic stirring to make the above described value Lx in the direction parallel to a long side of the mold a certain value or more. As a result of the examination on fluid simulation, which is described later, it was confirmed that the Lorentz force was not enough in a case where the current frequency was 0.4 Hz or less.

According to the above, it was assumed that there should exist the optimal current frequency between the current frequency where the above described value Lx in the direction parallel to a long side of the mold was maximum and the current frequency where electromagnetic stirring was improper. Numerical simulation on electromagnetic fields and fluid was examined to obtain this optimal current frequency.

Electromagnetic field simulation was carried out by calculating the distribution of the Lorentz force density generated in the molten steel by the electromagnetic stirrer according to the method as described above. Fluid simulation was carried out using the obtained Lorentz force density, to evaluate the number of bubbles of Ar gas captured by the solidified shell. Thermal fluid simulation was carried out according to the method described in Non Patent Literature 2, to calculate a flow of the molten steel, heat transmission, solidification and bubbles of Ar gas.

The thermal fluid simulation according to the method described in Non Patent Literature 2 make it possible to obtain information on the flow velocity, the speed of the solidification, the distribution of bubbles of Ar gas and so on in the molten steel in the continuous casting machine. Thus, the problem was how bubbles of Ar gas captured by the solidified shell were evaluated.

As described in Patent Literature 1, it is known that bubbles of Ar gas are not captured by the solidified shell if the flow velocity of the molten steel on the solidification interface is 10 to 60 cm/s. That is, calculation may be carried out assuming that in a case where the flow velocity of the molten steel on the solidification interface is the flow velocity where bubbles of Ar gas are captured (hereinafter referred to as the capture flow velocity) or below, bubbles of Ar gas existing on this location are captured.

Generally speaking, a threshold of the above capture flow velocity is 20 cm/s. However, the accurate value is unknown. In addition, it is considered to be unnatural that such calculation is carried out assuming that when the flow velocity of the molten steel is 19.9 cm/s, bubbles of Ar gas are not captured by the solidified shell and when the flow velocity thereof is 20.1 cm/s, the bubbles are captured thereby.

Thus, the inventor invented a method of evaluating the probability that bubbles of Ar gas were captured by the solidified shell as a continuous function as represented by the following formula (1). Here, P_{g}(-) is the probability that bubbles of Ar gas are captured by the solidified shell, C₀ is a fixed number, and U (m/s) is the flow velocity of the molten steel on the solidification interface.

In a case where the fixed number Co in the following formula (1) is 100, the capture probability P_{g} when the flow velocity of the molten steel is 20 cm/s is no more than 10⁻⁸. This is such probability that one of a million bubbles of Ar gas is captured by the solidified shell, and this value of the probability is considered to be 0 on numerical simulation. It is noted that any of 10 to 1000 is a proper value for Co used in numerical simulations.
[Math. 1] ${P}_{g} = exp \left(-{C}_{0}⋅U\right)$

The speed η_{g} (number/m³·s) where bubbles of Ar gas are captured by the solidified shell is represented as the following formula (2), with the number density n_{g} (number/m³) of bubbles of Ar gas on the solidification interface, the solidification speed Rₛ (1/s) and the capture probability P_{g}(-).
[Math. 2] ${η}_{g} = {n}_{g} ⋅ {R}_{s} ⋅ {P}_{g}$

The number density of bubbles of Ar gas in the solidified shell S_{g} (number/m³) is calculated from the following formula (3). Here, Uₛ is the movement speed (m/s) of the solidified shell in the slab drawing direction.
[Math. 3] $\frac{\partial {S}_{g}}{\partial t} + ∇ ⋅ \left({U}_{s}{S}_{g}\right) = {η}_{g}$

The number density S_{g} (number/m³) of bubbles of Ar gas in the solidified shell obtained from the above formula (3) was time-averaged, to evaluate the number of bubbles of Ar gas. At this time, it was considered that the capture flow velocity naturally varied according to diameters of bubbles of Ar gas, but the relationship therebetween is unknown. Then, the examination was carried out under the condition where each bubble of Ar gas existing mainly in the mold of the continuous casting machine is 1 mm in diameter. The evaluation was carried out within the range of 2 mm from the superficial slab, as a range where bubbles of Ar gas of 1 mm in diameter influenced on the surface of the slab.

FIG. 6 shows the results of examining the relationship between the current frequency and the number of pinholes per unit area (number/m²) on the solidification interface, based on numerical analysis.

It becomes clear from FIG. 6 that the number of pinholes in a case where the current frequency is 1.2 Hz is less than a case where the current frequency is 2.3 Hz, where the Lorentz force density is the maximum; and the number of pinholes largely increases as the current frequency is 0.8 Hz and below.

The reason why the number of pinholes per unit area on the solidification interface is the minimum, 43 (number/m²) in a case where the current frequency is 1.2 Hz is that while the Lorentz force density decreases due to electromagnetic stirring, the decrease of the electromagnetic repulsion produces a large effect of decreasing bubbles of Ar gas near the wall surface of the mold. However, pinholes increase as the current frequency decreases to 1.2 Hz and below because the Lorentz force density for stirring the molten steel in the mold is not enough.

Generally, the current frequency where the Lorentz force density is the maximum is selected for the current frequency of an electromagnetic stirrer. In the electromagnetic stirrer shown in FIG. 1, the current frequency where the Lorentz force density is the maximum is 2.3 Hz, which is read in FIG. 3. The number of pinholes in a case where the current frequency is 2.3 Hz, which is selected according to prior arts is 57 (number/m²) as shown in FIG. 6. Thus, as is seen from FIG. 6, pinhole defects can be suppressed more than prior arts at any current frequency within the range of 0.9 Hz to 2.3 Hz.

Therefore, the inventor obtained the knowledge under the conditions where the size of the slab was 1200 mm in width × 250 mm in thickness, the copper mold was 25 mm in thickness, and the conductivity of the copper mold was 1.9 × 10⁷ S/m, the proper range of the frequency where the number of pinholes can be suppressed more than conventional arts was 0.9 to 2.3 Hz.

It takes a relatively long time to carry out such fluid analysis for evaluating pinholes compared with electromagnetic field analysis. Thus, the inventor studied a method for selecting the optimal frequency from the result of electromagnetic field analysis.

The Lorentz force Lx (N/m³) necessary for electromagnetic stirring functions as a positive factor for the number of pinholes, and the electromagnetic repulsion Ly (N/m³) functions as a negative factor therefor. Therefore, effective Lorentz force density F (N/m³) is defined as represented by the following formula (4). Here, α is a coefficient that indicates bad influence of the electromagnetic repulsion.
[Math. 4] $F = Lx - α ⋅ Ly$

Since the above described α is a coefficient that indicates bad influence in the direction parallel to a short side of the mold, this influence varies according to the length of a short side of the mold. The inventor examined α with which the evaluation using the above formula (4) was equivalent to that shown in FIG. 6 concerning 200 mm to 300 mm of a short side of the mold in length as a common continuous casting machine. As a result, the inventor obtained the knowledge that α in the range of 3 to 7 is proper. In a case where α is less than 3, the Lorentz force parallel to a short side of the mold is underestimated, and in a case where α is beyond 7, the Lorentz force parallel to a short side of the mold is overestimated.

FIG. 7 shows frequency dependency of the effective Lorentz force density F (N/m³) in a case where the coefficient α that indicates bad influence of electromagnetic repulsion is 5. It is seen from FIG. 7 that the effective Lorentz force density F (N/m³) takes the maximum value in a case where the current frequency is 1.2 Hz.

In view of FIGS. 3 to 6, pinhole defects can be suppressed more than conventional arts in a case where the current frequency is within the range of 0.9 Hz to 2.3 Hz. This range corresponds to a range of the maximum value Fmax to 0.9 Fmax of the effective Lorentz force density F (the current frequency is in the range of 0.9 to 2.0 Hz). As described above, using the above formula (4) makes it possible to determine the best frequency of the electromagnetic stirrer only with the result of the electromagnetic field analysis.

The present invention was made based on the above results of inventor's studies, and is a method for continuously casting steel using a mold and an electromagnetic stirrer, the mold being equipped with the electromagnetic stirrer, the method comprising: obtaining a relationship between effective Lorentz force density F (N/m3) that is calculated by the above described Formula (4), and current frequency (Hz) of the electromagnetic stirrer, and using current frequency of the electromagnetic stirrer such that the effective Lorentz force density F is within a range of Fmax to 0.9 Fmax wherein Fmax is a maximum value of the effective Lorentz force density F, wherein Lx (N/m3) is an average value of Lorentz force density components in a direction parallel to a long side of the mold within existence of an iron core, the iron core being a component of the electromagnetic stirrer, and Ly (N/m3) is an average value of Lorentz force density components in a direction parallel to a short side of the mold within existence of the iron core.

According to the present invention described above, the best current frequency of the electromagnetic stirrer, where the electromagnetic repulsion generated when electromagnetic stirring is carried out on the molten steel in the mold can be made to be as little as possible can be determined only from the result of the electromagnetic analysis. Therefore, it can be suppressed as far as possible to gather bubbles of Ar gas on the superficial slab, and pinhole defects can be further suppressed.

While the inventor carried out fluid simulation with the method described in Non Patent Literature 2, it is needless to say that thermal fluid simulation can be carried out not only with the method described in Non Patent Literature 2 but also with another method.

### Reference Signs List

- 11: ... mold
- 13: ... electromagnetic stirrer
- 13a: ... iron core

## Claims

1. A method for continuously casting steel using a mold (11) and an electromagnetic stirrer (13), the mold (11) being equipped with the electromagnetic stirrer (13), the method comprising:
obtaining a relationship between effective Lorentz force density F (N/m³) that is calculated by the following formula, and current frequency (Hz) of the electromagnetic stirrer (13); and
using current frequency of the electromagnetic stirrer (13) such that the effective Lorentz force density F is within a range of Fmax to 0.9 Fmax, wherein Fmax is a maximum value of the effective Lorentz force density F,
wherein $F = Lx - α ⋅ Ly ,$
wherein Lx (N/m³) is an average value of Lorentz force density components in a direction parallel to a long side of the mold (11) within existence of an iron core (13a), the iron core (13a) being a component of the electromagnetic stirrer (13);
Ly (N/m³) is an average value of Lorentz force density components in a direction parallel to a short side of the mold (11) within existence of the iron core (13a); and
α is a coefficient indicating bad influence of electromagnetic repulsion, wherein α is within the range of 3 to 7.

## Patentansprüche

1. Verfahren zum kontinuierlichen Gießen von Stahl unter Verwendung einer Form (11) und eines elektromagnetischen Rührwerks (13), wobei die Form (11) mit dem elektromagnetischen Rührwerk (13) ausgestattet ist, wobei das Verfahren Folgendes umfasst:
Erhalten einer Beziehung zwischen wirksamer Lorentzkraftdichte F (N/m³), die durch die folgende Formel berechnet wird, und Stromfrequenz (Hz) des elektromagnetischen Rührwerks (13); und
Verwenden der Stromfrequenz des elektromagnetischen Rührwerks (13), sodass die wirksame Lorentzkraftdichte F innerhalb eines Bereichs von Fmax bis 0,9 Fmax liegt, wobei Fmax ein Maximalwert der wirksamen Lorentzkraftdichte F ist,
wobei $F = Lx - α ⋅ Ly ,$
wobei Lx (N/m³) ein Durchschnittswert von Lorentzkraftdichte-Komponenten in eine Richtung ist, die parallel zu einer langen Seite der Form (11) in Vorhandensein eines Eisenkerns (13a) ist, wobei der Eisenkern (13a) eine Komponente des elektromagnetischen Rührwerks (13) ist;
Ly (N/m³) ein Durchschnittswert von Lorentzkraftdichte-Komponenten in eine Richtung ist, die parallel zu einer kurzen Seite der Form (11) in Vorhandensein des Eisenkerns (13a) ist; und α ein Koeffizient ist, der schlechten Einfluss von elektromagnetischer Abstoßung anzeigt, wobei α innerhalb des Bereichs von 3 bis 7 liegt.

## Revendications

1. Procédé de coulage continu d'acier à l'aide d'un moule (11) et d'un agitateur électromagnétique (13), le moule (11) étant équipé de l'agitateur électromagnétique (13), le procédé comprenant :
l'obtention d'une relation entre la densité de force de Lorentz efficace F (N/m³) qui est calculée par la formule suivante, et une fréquence actuelle (Hz) de l'agitateur électromagnétique (13) ; et
l'utilisation de la fréquence actuelle de l'agitateur électromagnétique (13) de sorte que la densité de force de Lorentz efficace F se trouve dans une plage de Fmax à 0,9 Fmax, Fmax étant une valeur maximale de la densité de force de Lorentz efficace F,
où $F = Lx - α ⋅ Ly ,$
où Lx (N/m³) est une valeur moyenne de composantes de densité de force de Lorentz dans une direction parallèle à un côté long du moule (11) dans l'existence d'un noyau en fer (13a), le noyau en fer (13a) étant un composant de l'agitateur électromagnétique (13) ;
où Ly (N/m³) est une valeur moyenne de composantes de densité de force de Lorentz dans une direction parallèle à un côté court du moule (11) dans l'existence du noyau en fer (13a) ; et
α est un coefficient indiquant une mauvaise influence de la répulsion électromagnétique, α étant dans la plage de 3 à 7.
